

1

3,386,831

STABILIZING OF PHOTOGRAPHIC SILVER  
HALIDE EMULSIONS WITH ACYL PHEN-  
YL HYDRAZIDES

Hans Ludwig Honig, Leverkusen, Günter Kolb and Franz Moll, Cologne-Stammheim, and Bernhard Morcher, Leverkusen, Germany, assignors to Agfa Aktiengesellschaft, Leverkusen, Germany, a corporation of Germany  
No Drawing. Filed Feb. 24, 1965, Ser. No. 435,067  
Claims priority, application Germany, Mar. 5, 1964,  
A 45,411  
10 Claims. (Cl. 96—109)

The invention relates to photographic emulsions and particularly to a process for stabilizing photographic silver halide emulsions by the addition of phenylhydrazides of aliphatic carboxylic acids.

Silver halide emulsions prepared by the usual processes undergo a marked reduction in their sensitivity, a flattening in the graduation and increased fogging when stored under tropical conditions. The sensitivity nuclei and the latent image nuclei of exposed silver halide emulsions are not stable in storage. Stabilization of the latent image is of particular importance in multilayered color photography since the various additives in the individual layers, such as color components, sensitizers etc. cause varying degrees of alteration of the latent image on storage and thus cause a shift in the color balance.

It is known to add hydrazinium salts or hydrazine compounds to photographic silver halide emulsions, as described for instance in British Patent No. 598,106 for increasing the speed or contrast or both of such emulsions.

However, the hydrazine compounds customarily employed in photographic emulsions show practically no stabilizing effect. They have even been used for fogging silver halide emulsions to render reversal exposure of the material unnecessary. Moreover, many hydrazine compounds impair or even completely prevent hardening of the gelatin by ordinary hardening agents.

It is an object of the present invention to provide photographic silver halide emulsions, the latent image of which is stabilized. A further object is to provide a new method for stabilizing the latent image of photographic silver halide emulsions. Other objects will appear from the following description of our invention.

We now have found that the stabilization of the latent image specks and of the so-called sensitivity specks in particular of silver halide emulsions which are after-ripened and the latent image specks of which are situated essentially on the surface of the silver halide grain can be achieved even under extreme conditions of storage such as storage under tropical conditions by adding phenylhydrazides of aliphatic, saturated or unsaturated mono- or polycarboxylic acids having preferably up to 12 carbon atoms more particularly up to 5 carbon atoms per phenylhydrazide unit, to the photographic emulsions. The compounds are characterized in that they contain at least once the following group



wherein the phenyl nucleus can be substituted as desired by any groups that are photographically inert. These include, for preference, alkyl radicals having up to 5 C-atoms, alkoxy radicals, preferably of the same type as

2

the alkyl radicals, halogen atoms such as chlorine or bromine and carboxyl groups.

The group given in the above formula is linked to straight chained or branched, saturated or unsaturated aliphatic radicals.

The following compounds have been found suitable for use according to our invention:

- 5 acetic acid phenylhydrazide,
- 10 acetic acid-p-tolylhydrazide,
- 15 propionic acid phenylhydrazide,
- 20 butyric acid phenylhydrazide,
- 25 methacrylic acid phenylhydrazide,
- 30 isobutyric acid phenylhydrazide,
- 35 maleic acid-bis-phenylhydrazide,
- 40 fumaric acid-bis-phenylhydrazide,
- 45 itaconic acid-bis-phenylhydrazide,
- 50 glutaric acid-bis-phenylhydrazide,
- 55 citric acid-tri-phenylhydrazide,
- 60 polymethacrylic acid phenylhydrazide,
- 65 adipic acid-bis-phenylhydrazide.

The silver halide emulsions are produced in accordance with common practice. The preparation involves 3 separate steps: (1) precipitation of the silver halide and physical ripening in the presence of gelatin, (2) freeing of the emulsion of excess water-soluble salt usually by washing and (3) after-ripening or chemical ripening to obtain the desired speed or sensitivity.

The substances can be added at any desired stage to the light-sensitive silver halide emulsion layer or if desired to auxiliary layers.

In the preparation of the photographic emulsions of the present invention the phenylhydrazides are advantageously incorporated in the finished emulsion after the chemical ripening. It is convenient to add the stabilizers of the present invention from solutions in appropriate solvents. The solvent should, of course, be completely free from any deleterious effect on the silver halide emulsion. Water or lower aliphatic alcohols or admixtures thereof have proven satisfactory as solvents for the majority of the stabilizers of the invention. The concentration of the stabilizers in the emulsion can vary widely from about 0.1 to 20 g. per mol of silver halide, their specific concentration will vary according to the type of the light-sensitive emulsion and according to the effects desired. Preferred are concentrations of between 1 and 10 g. per mol of silver halide. The most suitable concentration for any given emulsion will be apparent upon making the test customarily used in the art.

It has surprisingly been found that while all the usual photographic properties are retained (these are determined largely by the structure of the silver halide emulsion), there is obtained in addition an excellent stabilization of the latent image specks. Even when the photographic materials produced by the process according to the invention are stored over a considerable period at normal temperature or under the conditions of high temperature and humidity which may occur in tropical climates for example, no fading of the latent image specks takes place.

The emulsions for which the phenylhydrazides according to the invention are used, are after-ripened in accordance with common practice. The emulsions essentially form a latent image on the surface of the silver halide grain.

The emulsions may contain the customarily employed

silver halides such as silver chloride, silver bromide or mixtures thereof, which may contain a small amount of about up to 10 mol percent of silver iodide. Suitable as binding agents for the light-sensitive layer are the usual hydrophilic binders such as carboxymethylcellulose, polyvinyl alcohol, vinyl pyrrolidone, alginic acid and its salts, esters or amides and especially gelatin.

The emulsions stabilized in accordance with the present invention can be chemically sensitized by any of the accepted procedures. The emulsions can be treated with salts of the noble metals such as ruthenium, rhodium, palladium, iridium and platinum. Suitable compounds are well known in the art. The emulsions can also be sensitized with gold salts as described by R. Koslowsky Z. wiss. phot. 46, 65-72 (1951). The emulsions can also be chemically sensitized with reducing agents such as stannous salts, polyamines, sulfur compounds, such as described in the U.S. Patent 1,574,944, polyethylene oxides and the like. The emulsions can also be optically sensitized with the ordinary sensitizing dyes, cyanines or merocyanines. The emulsions can be stabilized with any of the known stabilizers such as mercury compounds, triazoles, azaindenes, such as disclosed by Birr in Z. wiss. phot., vol. 47 (1952), pages 2-28. The emulsions may be hardened by any suitable hardener, such as formaldehyde and halogen-substituted aliphatic acids such as mucobromic acid.

#### Example 1

A highly sensitive silver iodobromide gelatin emulsion having an iodine content of 4 mols percent and a silver nitrate/gelatin ratio of 1:1 is produced by the usual method, washed and after-ripened to maximum sensitivity with the use of sulfur- and gold sensitizers.

The pH of the finished emulsion is 6.4. Before pouring onto the usual photographic surfaces, the customary stabilizers such as 200 mg. of 1,3,3a,7-tetraaza-4-hydroxy-6-methylindene per liter emulsion, wetting agents such as 30 ml. of a 7.5% aqueous solution of saponin per liter emulsion and hardening agents such as 15 ml. of a 10% aqueous formaldehyd solution per liter emulsion are added to the emulsion.

The above emulsion was divided into several portions and phenyl hydrazides of the present invention were added from aqueous or methanolic solution in the amounts indicated in the following table:

TABLE 1

| Sample: | Stabilizer                      | Amount per mol of silver halide, g. |
|---------|---------------------------------|-------------------------------------|
| A       |                                 |                                     |
| B       | Acetic acid phenylhydrazide     | 1.7                                 |
| C       | do                              | 3.4                                 |
| D       | Isobutyric acid phenylhydrazide | 1.7                                 |
| E       | do                              | 3.4                                 |
| F       | do                              | 6.8                                 |

The various portions of the emulsions were then coated on a transparent support, such as cellulose acetate and dried. The final light-sensitive layers contained about 7 g. of silver per square meter in the form of silver halide.

A part of the various samples was first stored for 7 days at 35° C. and 85% relative humidity while the other part was photographically processed in the fresh state. The photographic processing includes exposure in an ordinary sensitometer and development for about 5 minutes at 20° C. in a photographic developer having the following composition:

|                                       |     |
|---------------------------------------|-----|
| N-methyl-p-aminophenolsulfonate       | 3.5 |
| Sodium sulfite sicc.                  | 60  |
| Hydroquinone                          | 9   |
| Soda sicc.                            | 40  |
| Potassium bromide made up to 1000 ml. | 3.5 |

G.  
70  
75

The results of the sensitometer tests are shown in the following Table 2:

TABLE 2

| 5      | Sensi-<br>tivity | Fresh |           |    | Stored |           |  |
|--------|------------------|-------|-----------|----|--------|-----------|--|
|        |                  | Fog   | Gradation |    | Fog    | Gradation |  |
| Part A | 100              | 0.10  | 1.7       | 50 | 0.13   | 1.45      |  |
| Part B | 100              | 0.09  | 1.7       | 75 | 0.09   | 1.6       |  |
| Part C | 100              | 0.09  | 1.7       | 83 | 0.09   | 1.7       |  |
| Part D | 100              | 0.09  | 1.7       | 75 | 0.09   | 1.6       |  |
| Part E | 100              | 0.09  | 1.8       | 83 | 0.09   | 1.8       |  |
| Part F | 100              | 0.09  | 1.8       | 83 | 0.09   | 1.8       |  |

The melting point of the layers is above 100° C. in all the samples. As seen from the table, the substances according to the invention largely prevent reduction in the sensitivity and flattening of the gradation in storage at high temperature and humidity. They also decrease fog formation.

20

#### Example 2

Before casting, a silver halide gelatin emulsion was treated with 0.3 g. of chloromucic acid per kg. of emulsion and 3.4 g. per silver halide mol of the hydrazine compound given below. After casting, drying and 48 hours storage, the melting point of the layer was determined. The results are given in Table 3.

TABLE 3

| 30   | Substance added                                 | Melting point of the emulsion |
|------|-------------------------------------------------|-------------------------------|
| 1... | Without additive                                | Above 100° C.                 |
| 35   | 2... <chem>CH3-CO-NH-NH-C6H5</chem>             | Above 100° C.                 |
| 40   | 3... <chem>CH3-CH(CO-NH-NH-C6H5)-CH2-CH3</chem> | 32° C.                        |
| 45   | 4... <chem>CH3-CH(CO-NH-NH-CH2-C6H5)-CH3</chem> |                               |
| 50   | 5... <chem>CH3-CH(CO-NH-NH-C6H5)-CH3</chem>     |                               |
| 55   | 6... <chem>CH3-CH(CO-NH-N=C6H5)-CH3</chem>      |                               |

Whereas the phenyl substituted carboxylic acid hydrazides according to the invention given under (2) do not impair the hardening effect, hydrazides which have a free NH<sub>2</sub> group, alkyl-, cycloalkyl- and aralkyl-substituted hydrazides and acyl hydrazones prevent hardening of the gelatin. Compounds of the type given under (3) are therefore of limited utility as additives for photographic layers.

60

#### Example 3

Numerous hydrazine compounds which also do not prevent hardening of gelatin were added to a silver halide emulsion as described in Example 1 and their effect compared with phenylhydrazides according to the invention. Chloromucic acid was used as hardening agent. In all the samples, the melting point of the layer was above 100° C.

The results of the tests are shown in the following Table 4:

75

TABLE 4

| Substance added       | Quantity<br>in g. per<br>mol Ag | Fresh            |               |                | Stored           |                |                  |
|-----------------------|---------------------------------|------------------|---------------|----------------|------------------|----------------|------------------|
|                       |                                 | Sensi-<br>tivity | Fog           | Grad-<br>ation | Sensi-<br>tivity | Fog            | Grad-<br>ation   |
| Without additive..... |                                 | 100              | 0.10          | 1.7            | 50               | 0.13           | 1.4 <sup>1</sup> |
|                       | 1.7<br>3.4                      | 100<br>100       | 0.09<br>0.09  | 1.7<br>1.7     | 75<br>83         | 0.09<br>0.09   | 1.6<br>1.7       |
|                       | 1.7<br>3.4                      | 100<br>100       | 0.09<br>0.09  | 1.8<br>1.8     | 75<br>83         | 0.09<br>0.09   | 1.8<br>1.8       |
|                       | 1.7<br>3.4                      | 100<br>100       | 0.11<br>0.11  | 1.6<br>1.4     | 50<br>50         | 0.13<br>0.15   | 1.45<br>1.3      |
|                       | 1.7<br>3.4                      | 100<br>100       | 0.09<br>0.09  | 1.8<br>1.8     | 50<br>66         | 0.12<br>0.12   | 1.8<br>1.8       |
|                       | 1.7<br>3.4                      | 100<br>100       | 0.10<br>0.10  | 1.4<br>1.5     | 50<br>42         | 0.13<br>0.13   | 1.25<br>1.4      |
|                       | 1.7<br>3.4                      | 100<br>100       | 0.10<br>0.10  | 1.9<br>1.7     | 50<br>50         | 0.13<br>0.11   | 1.8<br>1.8       |
|                       | 1.7<br>3.4                      | 100<br>100       | 0.09<br>0.10  | 1.8<br>1.8     | 50<br>50         | 0.13<br>0.13   | 1.7<br>1.7       |
|                       | 1.7<br>3.4                      | 100<br>100       | 0.08<br>0.08  | 1.8<br>1.8     | 50<br>66         | 0.12<br>0.12   | 1.7<br>1.7       |
|                       | 1.7<br>3.4                      | 200<br>(1)       | 0.80<br>----- | 0.8<br>-----   |                  | Black<br>Black |                  |
|                       | 1.7<br>3.4                      | 100<br>100       | 0.10<br>0.11  | 1.5<br>1.5     |                  | Black<br>Black |                  |
|                       | 1.7<br>3.4                      | 100<br>117       | 0.13<br>0.13  | 1.6<br>1.7     |                  | Black<br>Black |                  |

<sup>1</sup> Strong fogging.

The above table shows that only the phenylhydrazides of the present invention stabilize the latent image specks or the sensitivity of the silver halide emulsion. Other phenylhydrazides either have no stabilizing effect or cause a strong fogging of the silver halide emulsion layers.

## Example 4

A multilayer colorphotographic element is produced which includes a blue-sensitive silver halide emulsion layer containing 3-(p-stearyl-aminobenzoyl-acetamino) - isophthalic acid as yellow coupler, a green-sensitive silver halide emulsion layer containing 1-(3'-sulfo-4'-phenoxy)-phenyl-3-heptadecyl-pyrazolone-(5) as magenta coupler and a red-sensitive silver halide emulsion layer containing 1-hydroxy - 2 - naphthoic acid-(2'-(methyl-n-octadecylamino)-5'-sulfonic acid)-anilide as cyan coupler. The silver halide of the three light-sensitive layers essentially consists of silver bromide. In addition to these couplers, the usual casting additives as described by Glafkides: Photographic Chemistry, vol. 2 (Fountain Press, London), pages 564-568 for reverse color films are added to the three layers (Sample I).

A second multilayer colorphotographic element is produced in the same way but 100 ml. of a 1% aqueous solution of acetic acid phenyl hydrazide is added per kg. of the emulsion containing the yellow coupler before the upper layer is cast (Sample II).

Both films are exposed behind a grey step wedge and stored for 8 weeks at about 20° C. and relative humidity of about 65%.

Two further identical samples of the two photographic elements were produced and in the fresh state are exposed under the identical conditions. The exposed samples are then subjected to a reverse development in accordance with common practice. Suitable baths and conditions are described by Glafkides "Photographic Chemistry," vol. 2, pages 631-632.

TABLE 5

| 55      | Sample | Fresh        |       | Stored      |            |
|---------|--------|--------------|-------|-------------|------------|
|         |        | Sensitivity  | Color | Sensitivity | Color      |
| I.....  | 100    | Neutral..... | ..... | 50          | Yellowish. |
| II..... | 100    | do.....      | ..... | 85          | Neutral.   |

60 The blue-sensitive emulsion layer was particularly subject to fading with respect to the latent image specks. This is clearly apparent from the yellowish color of the stored Sample I, which have a yellowish tint because of the reversal development. With stabilized Sample II a neutral grey image is obtained.

65 The phenylhydrazides utilized in accordance with the present invention are prepared by the conventional methods for the production of hydrazides of carboxylic acid. Suitable methods are disclosed in the handbook "Methoden der organischen Chemie" by Houben-Weyl, 4th edition, volume 8, Part III, pages 676-680, published by Georg Thieme Verlag, Stuttgart 1952.

We claim:

70 1. An after-ripened photographic silver halide emulsion the silver halide grains of which are essentially sur-

face-sensitive and which contains a stabilizing amount of a  $\beta$ -mono-phenylhydrazide of an aliphatic carboxylic acid.

2. A photographic silver halide emulsion as defined in claim 1 in which the carboxylic acid is a mono-carboxylic acid.

3. A photographic silver halide emulsion as defined in claim 1, wherein the phenylhydrazide is characterized by the following formula:



wherein:

R is an aliphatic radical having up to 6 carbon atoms of the groups consisting of saturated alkyl and olefinically unsaturated alkyl, y stands for a whole number from 1 to 3 and

X represents a substituent of the group consisting of hydrogen, alkyl, alkoxy, halogen and carboxyl.

4. A photographic silver halide emulsion as defined in claim 3, in which the phenylhydrazide is the  $\beta$ -mono-phenylhydrazide of acetic acid.

5. In a process of making photographic images including the steps of exposing to the object to be reproduced a photographic element comprising a supported light-sensitive silver halide emulsion layer, developing and fixing the exposed element, the improvement consisting of performing the process with a photographic element containing a stabilizing amount of a  $\beta$ -mono-phenylhydrazide of an aliphatic carboxylic acid.

6. A process as defined in claim 5, wherein the carboxylic acid is a monocarboxylic acid.

7. A process as defined in claim 6, wherein the phenylhydrazide has the formula



wherein:

R is an aliphatic radical having up to 6 carbon atoms of the group consisting of saturated alkyl and olefinically unsaturated alkyl and

5 X represents a substituent of the group consisting of hydrogen, alkyl, alkoxy, halogen and carboxyl.

8. A process as defined in claim 7, wherein R is methyl.

9. A photographic silver halide emulsion containing from about 0.1 to about 20 grams per mole silver halide of a substituted or unsubstituted  $\beta$ -mono-phenylhydrazide of an aliphatic carboxylic acid, said  $\beta$ -mono-phenylhydrazide when substituted having a phenyl substituent selected from the group consisting of alkyl having up to 5 carbon atoms, alkoxy having up to 5 carbon atoms, halogen and carboxyl and said aliphatic carboxylic acid being a mono-carboxylic or polycarboxylic, saturated or unsaturated acid.

10. A method of stabilizing the latent image specks in a photographic silver halide emulsion comprising adding to said photographic silver halide emulsion from about 0.1 to about 20 grams per mole silver halide of a substituted or unsubstituted  $\beta$ -mono-phenylhydrazide of an aliphatic carboxylic acid, said  $\beta$ -mono-phenylhydrazide when substituted having a phenyl substituent selected from the group consisting of alkyl having up to 5 carbon atoms, alkoxy having up to 5 carbon atoms, halogen and carboxyl and said aliphatic carboxylic acid being a mono-carboxylic or polycarboxylic, saturated or unsaturated acid.

No references cited.

35 NORMAN G. TORCHIN, *Primary Examiner.*

J. R. EVERETT, *Assistant Examiner.*